# EUROPEAN PATENT SPECIFICATION

(11) **EP 1 573 148 B1**
(45) Date of publication and mention of the grant of the patent: **13.07.2011**
(21) Application number: 03813709.7
(22) Date of filing: 24.03.2003
(51) Int. Cl.: E04D 11/02

(54) **METHOD FOR PRODUCING A CONTINUOUS WATERPROOFING FLOORING**
VERFAHREN ZUR HERSTELLUNG EINES DURCHGEHENDEN WASSERSPERRBODENBELAGS
PROCEDE DE REALISATION DE COUCHE CONTINUE D'ETANCHEIFICATION DES SOLS

(30) Priority: 20.12.2002 IT TV20020054 U
(43) Date of publication of application: 14.09.2005
(73) Proprietor: Nord Resine S.p.A., 31058 Susegana (IT)
(72) Inventor: CAREGNATO, Lionello, I-31053 Pieve di Soligo (IT)
(86) International application number: PCT/IT2003/000170
(87) International publication number: WO 2004/057128

(56) References cited:
- EP-A- 0 794 299
- JP-A- 56 022 685

## Description

Nowadays, in the building industry, the waterproofing of flat roofs, terraces, balconies and the like is performed by various methods, which can be distinguished according to the chemical nature of the covering. We'll now briefly analyse the performances of such covering in order to highlight those limitations which can be overcome by the present invention.

### Bitumen-based waterproofing sheets

Bitumen-based waterproofing sheets are usually fixed to the roof by means of flame heating or self-adhesive systems. During manufacturing they can be coated with protective elements, as foils or coloured marble chips. These elements improve the appearance, the weatherability, the wear resistance and the tear resistance of the sheet. Nevertheless this material can't be considered a pedestrian or vehicle-suitable floor coating because of thermoplastic behaviour of bitumen with increasing temperature; in the summer, indeed, bitumen-based sheets, even though protected, are damaged and deformed by pedestrian or vehicle traffic. This material, moreover, is not water vapor permeable, so that it's impossible also for very small amount of liquid water to evaporate from foundation.

### Polyvinylchloride-based and olefinic rubber-based waterproofing sheets

This material is made of very wide prefabricated rolled up sheets and it's sufficient to lay them on the roof, without any adhesive system, and cover them with gravel or earth to prevent any movement. But if you want to make a concrete or tile flooring on this waterproofing material, you have not negligible additional cost due to the high cost of manual labour. Furthermore, neither of these sheets possess enough water vapor permeability to allow even the slightest percentage of water evaporation from foundation.

Resin-based waterproofing materials (two-component elastomeric polyurethane, one-component urethane, two-component epoxypolyurethane, polyester, two-component silicone resins and neoprene resins)

These materials possess characteristics of application that get close to the subject matter of the present invention; however, they show the following disadvantages:
i) insufficient water vapor permeability to allow application on wet foundation (if applied at this condition, bubble forming and detachment of the resin coating from the lower layer will occur);
ii) high cost of raw materials;
iii) need of applying more than one coating of resin and aggregates, thus increasing manual labour cost;

### Flexible two-component methacrylic resin-based waterproofing materials

These materials possess characteristics of application that get close to the subject matter of the present invention; however, they show the following disadvantages:
i) difficulties of application on very porous foundation (these materials are not fit to permeate and strengthen surfaces that will eventually have little cohesion);
ii) high cost of raw materials;
iii) high flammability of the components;
iv) high vapor pressure of the methacrylic monomer which implies a remarkable spreading of vapor and smell in the building site and the surroundings;
v) a marked tendency of the coating to yellowing.

Latex-based waterproofing membranes (acrylic esters, styrene-acrylate, and acrylonitrile latices)

These materials are a considerable part of the liquid applied waterproofing products in today's market. They show the following disadvantages:
i) insufficient permeability to water vapor to allow application on wet foundation (if applied on these conditions, bubble forming and detachment from foundation will occur);
ii) minimum film forming temperature higher than +7 + +8 °C;

### Liquid applied waterproofing membranes based on cement-latex mix

These materials are constituted by a powder part containing a cement binder, and by a conveniently formulated liquid part containing polymeric latices. The waterproofing system thus obtained guarantees the permeability to water vapor and the impermeability to liquid water, but it cannot be considered flooring system since it does not possess enough aesthetic characteristics and tear resistance; therefore it is necessary to apply a protective finish (e.g. tile covering).

There are patents that deal with continuous waterproofing covering systems and refer to the use of materials and to the limitations above mentioned.

Accordingly, mention is made of US 4,588,458, which discloses the use of a waterproofing membrane composed by a fibrous reinforcing base layer or matting impregnated with thermoplastic polymers-bitumen mix; GB 2193153, which discloses the use of a water vapor permeable felt constituted by non-woven fabric impregnated with bitumen on whose underside a film of perforated plastic material is applied, and then a thin metal layer; US 4,897,313, which discloses the use of a waterproofing system composed by a first coating of butyl acrylate, styrene and acrylonitrile copolymer latex, and a prefabricated self-adhesive sheet of bitumen modified with elastic polymers; WO 01/72514, which discloses the use of covering panels composed by an upper coating of acrylonitrile, styrene and acrylic esters copolymers and of a lower coating of polyvinylchloride; US 5,422,179, which discloses the use of waterproofing polymeric sheets obtained by copolymerization of ethylene, vinyl esters and acrylic esters; DE 3342560, which discloses the use of waterproofing sheets made of olefinic rubber strengthened with a fibreglass matting; US 6,395,845, which discloses the use of epoxy resin-based waterproofing sheets; WO 94/04349, which discloses the use of flexible protective waterproofing sheets composed by a flexible polymeric foil impregnated with a cement binder-based material; EP 0794299, in which a reference is made about production method of flat covering can be obtained by applying two coatings of a cement binder-latex mix reinforced, in the middle, by a perforated polypropylene sheet.

A principal aim of the present invention is therefore to solve the described problems, eliminating the drawbacks of the mentioned prior art, by providing a method that allows the production of a continuous waterproofing flooring on flat roofs, terraces, balconies and other flat structures.

Within the scope of this aim, an important object of the present invention is to provide a continuous waterproofing flooring that can be applied on any surface, new or old, constituted by cement foundation, different kinds of tiles or natural and artificial stone coverings.

Another object of the present invention is to provide a continuous waterproofing flooring that can be applied even on wet foundation and with temperatures down to +0.5 °C.

Another object of the present invention is to provide a continuous waterproofing flooring suitable for pedestrian and light vehicle use (with mass up to 3.5 tons), self-cleaning, nonslip, not subject to yellowing, wear and tear resistant.

Another object of the present invention is to provide a continuous waterproofing flooring that can be produced on site and in only two steps with a short interval of time between them.

This aim, these objects and others which will become apparent hereinafter are achieved by providing a method for producing a continuous waterproofing flooring, characterized in that it comprises the following steps:
a) a first step consists in laying a first layer, said laying of said first layer consists in laying, on a previously prepared foundation, a composite system formed by a prefabricated fibrous reinforcing base layer or matting, said prefabricated fibrous reinforcement base layer or matting being impregnated by a two-component liquid applied mix based on polymer latices and hydraulic binders;
b) a second step consisting in laying a second layer, said laying of said second layer consists in coating the above described first layer with a mix of polymers and additives, with or without any kind of aggregates, so as to create the visible side of the walkable and vehicle-suitable flooring.

Further characteristics and advantages of the invention will become apparent evident from the following detailed description of a particular structure thereof, illustrated only by way of non-limitative example in the accompanying drawings, wherein:
figure 1 is a perspective view of the flooring;
figure 2 is a sectional view of the flooring of figure 1.

With reference to the above figures, the reference numeral 1 designates a continuous waterproofing flooring for a previously prepared foundation 2 that is constituted by a base provided for example by means of a concrete casting.

The continuous waterproofing flooring is produced on site and entails the execution of both the above mentioned steps.

The first step consists in laying the layer 3 (two-component liquid applied waterproofing membrane based on a hydraulic binder-latex mix) on foundation 2. The two-component liquid applied waterproofing membrane based on a hydraulic binder-latex mix is composed of a mix of aggregates, additives, hydraulic binders, polymer latices and water obtained by mixing the dry and liquid components. Therefore the resulting material is composed of a mix of water, hydraulic binders and at least one polymer latex, for example styrene-acrylic esters latex. If necessary, just after the application of layer 3 is completed, you can proceed to lay a fibrous reinforcing base layer or matting 4 that can be constituited by non-woven fabric, felt, matting or any other structure that allows impregnation by and incorporation in layer 3; in this case it is advisable to lay on the fibrous reinforcing base layer or matting 4 a finishing layer 5 made of the same liquid mix. The interposition of the fibrous reinforcing base layer or matting 4 between the two layers of liquid mix allows to increase the tensile-strength characteristics of layer 3 and it should not alter the water vapor permeability of the system. Layers 3, 4 and 5 all together are waterproofing and water vapor permeable, so as to allow the laying of the system even on wet foundation. These characteristics are provided only by layer 3 when the liquid mix is applied without the fibrous reinforcing base layer or matting 4.

The second step consists in laying, on layer 5 (or 3, if the fibrous reinforcing base layer or matting 4 is not present), a pigmented or transparent mix of polymers and additives characterized by high water vapor permeability; this mix could eventually contain natural or artificial, coloured or not, aggregates.

The system obtained by laying the different components as described in the first and the second step, is the continuous waterproofing flooring, that is the object of the present invention.

The dimensions constituting the individual components of the product obtained with the present method can of course be the most appropriate according to the specific requirements.

Obviously, the method provided by the present invention is susceptible of changes, all of them being within the same inventive concept as defined by the appended claims.

## Claims

1. A method for producing a continuous waterproofing flooring obtainable exclusively by coupling two distinct layers, said method comprising the laying steps hereafter specified:
1.a) a first step consists in laying a first layer (3+4+5), said laying of said first layer (3+4+5) consists in laying, on a previously prepared foundation (2), a composite system formed by a prefabricated fibrous reinforcing base layer (4) or matting (4), said prefabricated fibrous reinforcement base layer (4) or matting (4) being impregnated by a two-component liquid applied mix based on polymer latices and hydraulic binders (3,5);
1.b) a second step consisting in laying a second layer (6), said laying of said second layer (6) consists in coating the above described first layer (3+4+5) with a mix of polymers and additives, with or without any kind of aggregates, so as to create the visible side of the walkable and vehicle-suitable flooring

2. A method according to claim 1, **characterized in that** said impregnating two-component liquid applied mix (3,5) of the composite system is composed by at least one polymer latex and one hydraulic binder.

3. A method according to claim 1, **characterized in that** the first layer (3+4+5) has the ability to bridge the cracks in the foundation without losing its waterproofing ability.

4. A method according to claim 1, **characterized in that** said impregnating two-component liquid applied mix (3,5) of the composite system acts as a waterproofing agent for the foundation.

5. A method according to claim 1, **characterized in that** said impregnating two-component liquid applied mix (3,5) of the composite system makes the prefabricated fibrous reinforcing base layer or matting adhere to the foundation.

6. A method according to claim 1, **characterized in that** said prefabricated fibrous reinforcing base layer (4) or matting (4) can be made of non-woven fabric, felt, , or matting.

7. A method according to claim 1, **characterized in that** at least one component of the coating (6), constituting the visible side of the walkable and vehicle-suitable flooring, is an acrylic polymer.

8. A method according to claim 1, **characterized in that** at least one component of the coating (6), constituting the visible side of the walkable and vehicle-suitable flooring, is a styrene-acrylic ester copolymer.

9. A method according to claim 1, **characterized in that** at least one component of the coating (6), constituting the visible side of the walkable and vehicle-suitable flooring, is an epoxy polymer.

10. A method, according to claim 1, **characterized in that** at least one component of the coating (6), constituting the visible side of the walkable and vehicle-suitable flooring, is a methacrylic polymer.

11. A method according to claim 1, **characterized in that** at least one component of the coating (6), constituting the visible side of the walkable and vehicle-suitable flooring, is an unsaturated polyester resin.

12. A method according to claim 1, **characterized in that** at least one component of the coating (6), constituting the visible side of a walkable and vehicle-suitable flooring, is a polyurethane resin.

13. A method according to claim 1, **characterized In that** the polymer resins in the coating (6), constituting the visible side of the walkable and vehicle-suitable flooring, can be transparent, coloured or pigmented.

## Patentansprüche

1. Ein Verfahren zur Herstellung einer kontinuierlichen Fußboden-Versiegelung durch eine exklusive Verbindung von zwei unterschiedlichen Schichten, wobei das Verfahren und die notwendigen Schritte nachstehend beschrieben werden:
1.a) Der erste Schritt besteht aus der Verlegung einer ersten Schicht (3 +4 +5), wobei die Schicht der obersten Ebene (3 +4 +5) genannt wird und aus der Verlegung auf einem zuvor hergestellten Untergrund (2) besteht. Ein zusammengesetztes System, das aus einer Grundschicht mit Faserverstärkung (4) oder Matten (4) besteht und mit einer Mischung aus einer Zwei-Komponenten-Flüssigkeit mit polymerem Latex und hydraulischen Bindemitteln (3, 5) imprägniert wird;
1.b) Der zweite Schritt besteht aus der Verlegung einer zweiten Schicht (6), wobei diese zweite Schicht (6) aus der Beschichtung der oben beschriebenen ersten Schicht (3 +4 +5) mit einer Mischung von Polymeren und Additiven besteht, mit oder ohne jeder Art von Aggregaten, um so die sichtbare Seite des begehbaren und mit Fahrzeugen befahrbaren Bodenbelages zu schaffen.

2. Das Verfahren nach Anspruch 1 ist **dadurch gekennzeichnet, dass** die imprägnierende Zweikomponenten-Flüssigkeit der aufgetragenen Mischung (3,5) aus dem Verbindungssystem mit mindestens einem Polymer Latex und einem hydraulischen Bindemittel besteht.

3. 3Das Vorfahren nach Anspruch 1 besteht in der Charakteristik, indem die erste Schicht (3 +4 +5) die Fähigkeit besitzt, die Risse im Fundament zu überbrücken, ohne seine Fähigkeit der Wasserdichte zu verlieren.

4. Das Verfahren nach Anspruch 1 ist **dadurch gekennzeichnet, dass** die imprägnierende zweikomponenten-Flüssigkeitsmischung (3,5) des Verbindungssystems als wasserdichtes Mittel für den Untergrund dient.

5. Das Verfahren nach Anspruch 1, ist **dadurch gekennzeichnet, dass** die imprägnierende Zweikomponenten-Flüssigkeitsmischung (3,5) des zusammengesetzten Systems die vorgefertigte faserige Verstärkungssehicht oder Matten fest am Untergrund haften lässt.

6. Das Verfahren nach Anspruch 1 ist **dadurch gekennzeichnet, dass** das genannte faserige Verstärkungsmaterial der Basisschicht (4) oder Matten (4) aus nicht gewobenen Stoff hergestellt werden kann, Stoff oder Matten.

7. Das Verfahren nach Anspruch 1 ist **dadurch gekennzeichnet, dass** mindestens eine Komponente der Beschichtung (6), aus dem die sichtbare Seite des begehbaren und mit Fahrzeugen befahrbarem Bodenbelages besteht, ein Acryl-Polymer ist.

8. Das Verfahren nach Anspruch 1 ist **dadurch gekennzeichnet, dass** mindestens eine Komponente der Beschichtung (6), aus dem die sichtbare Seite des begehbaren und mit Fahrzeugen befahrbarem Bodenbelages besteht, ein Styrol-Acrylester-Copolymer ist.

9. Das Verfahren nach Anspruch 1 ist **dadurch gekennzeichnet, dass** mindestens eine Komponente der Beschichtung (6), aus dem die sichtbare Seite des begehbaren und mit Fahrzeugen befahrbarem Bodenbelages besteht, ein Polymer aus Epoxidharz ist.

10. Das Verfahren nach Anspruch 1 ist **dadurch gekennzeichnet, dass** mindestens eine Komponente der Beschichtung (6), aus dem die sichtbare Seite des begehbaren und mit Fahrzeugen befahrbarem Bodenbelages besteht, ein Methacrylpolymer ist.

11. Das Verfahren nach Anspruch 1 ist **dadurch gekennzeichnet, dass** mindestens eine Komponente der Beschichtung (6), aus dem die sichtbare Seite des begehbaren und mit Fahrzeugen befahrbarem Bodenbelages besteht, ein ungesättigter Polyesterharz ist.

12. Das Verfahren nach Anspruch 1 ist **dadurch gekennzeichnet, dass** mindestens eine Komponente der Beschichtung (6), aus dem die sichtbare Seite des begehbaren und mit Fahrzeug befahrbarem Bodenbelages besteht, ein Polyurethan-Harz ist.

13. Das Verfahren nach Anspruch 1 ist **dadurch gekennzeichnet, dass** die Polymer-Harze der Beschichtung (6), aus dem die sichtbare Seite des begehbaren und mit Fahrzeugen befahrbarem Bodenbelages besteht, transparent, farbig oder pigmentiert sein können.

## Revendications

1. Une méthode pour la production d'un sol imperméabilisé uniforme qui peut s'obtenir exclusivement en associant deux couches distinctes, ladite méthode comprenant les étapes des couches est spécifiées ci-après:
1.a) une première étape consiste à déposer une première couche (3+4+5), ladite pose de la première couche (3+4+5) consiste à la déposition sur une base préparée précédemment (2) d'un système composite formé par une couche de base renforcée de fibres préfabriquées (4) ou tapis (4) imprégné d'un liquide à double composant basé sur un mélange de latex polymère et de liants hydrauliques (3,5) ;
1.b) une seconde étape consiste en la déposition d'une seconde couche (6), ladite pose de la seconde couche (6) consiste en un revêtement de la première couche décrite ci-dessus (3+4+5) avec un mélange de polymères et d'additifs, avec ou sans agrégats, de telle sorte à créer la face visible du sol piétinnable et adaptable au véhicule.

2. Une méthode selon la revendication 1, **caractérisée par** ladite imprégnation d'un mélange liquide à double composant (3,5), du système composite se compose d'au moins un latex polymère et d'un liant hydraulique.

3. Une méthode selon la revendication 1, **caractérisée par** ladite première couche (3+4+5), a la possibilité de combler les fissures dans la fondation sans perte d'imperméabilité.

4. Une méthode selon la revendication 1 du système composite, **caractérisée par** ladite imprégnation du mélange à double composant liquide (3,5), agit en tant qu'agent imperméabilisant de la fondation.

5. Une méthode selon la revendication 1 du système composite, **caractérisée par** ladite imprégnation du mélange à double composant liquide (3,5), rend la couche de base renforcée de fibre préfabriquée ou tapis adhérant à la fondation.

6. Une méthode selon la revendication 1, **caractérisée par** ladite couche de base renforcée de fibre préfabriquée (4) ou tapis (4), peut être de tissu non-tissé, du feutre ou du tapis.

7. Une méthode selon la revendication 1, **caractérisée par** au moins un composant de revêtement (6), constituant la face visible du sol piétinnable et adapte au véhicule, est un polymère acrylique.

8. Une méthode selon la revendication 1, **caractérisée par** au moins un composant de revêtement (6), constituant la face visible du sol piétinnable et adapte au véhicule, est un copolymère styrène-ester acrylique.

9. Une méthode selon la revendication 1, **caractérisée par** au moins un composant de revêtement (6), constituant la face visible du sol piétinnable et adapte au véhicule, est un polymère époxy.

10. Une méthode selon la revendication 1, **caractérisée par** au moins un composant de revêtement (6), constituant la face visible du sol piétinnable et adapte au véhicule, est un polymère méthacrylique.

11. Une méthode selon la revendication 1, **caractérisée par** au moins un composant de revêtement (6), constituant la face visible du sol piétinnable et adapte au véhicule, est une résine polyester insaturé.

12. Une méthode selon la revendication 1, **caractérisée par** au moins un composant de revêtement (6), constituant la face visible du sol piétinnable et adapte au véhicule, est une résine polyuréthane.

13. Une méthode selon la revendication 1, **caractérisée par** au moins un composant de revêtement (6), constituant la face visible du sol piétinnable et adapte au véhicule, est transparent, en couleur ou à pigments.
